

# UNITED STATES PATENT OFFICE.

PAUL C. SEEL, OF ROCHESTER, NEW YORK, ASSIGNOR TO EASTMAN KODAK COMPANY,  
OF ROCHESTER, NEW YORK, A CORPORATION OF NEW YORK.

## BASE FOR ANTISTATIC FILM AND COMPOSITION FOR MAKING THE SAME.

1,415,059.

Specification of Letters Patent.

Patented May 9, 1922.

No Drawing. Original application filed December 31, 1920, Serial No. 434,354. Divided and this application filed April 16, 1921. Serial No. 461,916.

*To all whom it may concern:*

Be it known that I, PAUL C. SEEL, a citizen of the United States of America, residing at Rochester, in the county of Monroe 5 and State of New York, have invented certain new and useful Improvements in Bases for Antistatic Films and Composition for Making the Same, (Case B,) of which the following is a full, clear, and exact specification.

This invention relates to a base or support for anti-static photographic film and a composition for preparing such base. The principal object of my invention is to provide a support containing certain anti-static ingredients. Another object of my invention is to provide a suitable film-forming dope or composition for making such base or support. Other objects will hereinafter 20 appear.

I have found that photographic film may be rendered substantially anti-static by incorporating in the nitrocellulose base or support thereof certain substances together 25 with small amounts of water. The preferred substances which I employ are glucose and glycerin. In place of the glucose analogous sugary substances may be employed and in place of the glycerin I may 30 employ similar organic compounds of low volatility which are hygroscopic or have a strong affinity for water and are substantially inert toward the photographic coatings.

In practice I mix the anti-static ingredients together and then add such mixture to any of the usual nitrocellulose film dopes. In the preferred embodiment of my invention I add an amount of glucose equal to 40 from 2 to 4% of the weight of the nitrocellulose in the dope, an amount of glycerin equal to from 2 to 4% of the weight of the nitrocellulose in the dope and an amount of water equal to from 2 to 4% of the weight 45 of the nitrocellulose in the dope. Of course, these proportions are merely illustrative and may be varied considerably according to the thickness of the dope and the methods of spreading and curing the latter. But the 50 preferred proportions herein described operate well under the standard film-making conditions.

As an illustration of the formula to which my anti-static mixture may be added the

following is noted: 100 parts of nitrocellulose, 200 to 400 (say 250) parts of acetone, 200 to 400 (say 250) parts of methyl alcohol, 20 to 200 (say 40) parts of fusel oil. To this may be added, if desired, 1 to 30 (say 10) parts of camphor. My mixture of 4 parts of glucose, 4 parts of glycerin and 4 parts of water is then incorporated thoroughly in the dope.

The ingredients are those commonly used in the art, of sufficient purity to yield films 65 of the desired transparency and relative freedom from color. Various volatile solvents may be used and either acetone or methyl alcohol can be used alone in a suitable amount or varying mixtures can be employed. For the fusel oil may be substituted 70 the other monohydroxy aliphatic alcohols of from 4 to 5 carbon atoms, like normal butyl and isobutyl alcohols.

The dope is spread and cured by the 75 evaporation of the volatile solvents, so as to form a transparent flexible sheet or film base in the usual way. On this support the sensitive photographic coatings or emulsions are applied and from the product motion 80 picture films and other films are prepared as is well understood in the art. Such films are notably resistant to defects from the electrical discharges. While I am inclined to attribute this property to the increased electrical conductivity of the film 85 base, due to the moisture which is trapped or held therein by the glucose and glycerin, a knowledge of the theoretical basis of my invention is not necessary to the practicing 90 of it, as hereinabove described. It should be noted that the water, when incorporated with the substances and in the manner set forth in the examples given above, does not segregate in the film so as to impair the 95 transparency of the latter.

This case is a division of my application Serial No. 434,354, filed Dec. 31, 1920.

Having thus described my invention, what I claim as new and desire to secure by Letters Patent is:

1. A flexible transparent nitrocellulose base or support adapted to receive sensitive photographic coatings which contains a sugar, an inert hygroscopic organic compound of 105 low volatility and water.

2. A flexible transparent nitrocellulose base or support adapted to receive sensitive

photographic coatings which contains a sugar, glycerin and water.

3. A flexible transparent nitrocellulose base or support adapted to receive sensitive 5 photographic coatings which contains glucose, an inert hygroscopic organic compound of low volatility and water.

4. A flexible transparent nitrocellulose base or support adapted to receive sensitive 10 photographic coatings which contains glucose, glycerin and water.

5. A flexible transparent nitrocellulose base or support adapted to receive sensitive 15 coatings which contains an amount of a sugar equal to approximately 4% or less of the weight of the nitrocellulose, an amount of an inert hygroscopic organic compound of low volatility equal to substantially 4% or less of the weight of the nitrocellulose 20 and an amount of water equal to substantially 4% or less of the weight of the nitrocellulose.

6. A flexible transparent nitrocellulose base or support adapted to receive sensitive 25 coatings which contains an amount of a sugar equal to approximately 4% or less of the weight of the nitrocellulose, an amount of glycerin equal to substantially 4% or less of the weight of the nitrocellulose and an 30 amount of water equal to substantially 4% or less of the weight of the nitrocellulose.

7. A flexible transparent nitrocellulose base or support adapted to receive sensitive 35 coatings which contains an amount of glucose equal to substantially 4% or less of the weight of the nitrocellulose, an amount of an inert hygroscopic organic compound of low volatility equal to substantially 4% or less of the weight of the nitrocellulose and 40 an amount of water equal to substantially 4% or less of the weight of the nitrocellulose.

8. A flexible transparent nitrocellulose base or support adapted to receive sensitive 45 coatings which contains an amount of glucose equal to substantially 4% or less of the weight of the nitrocellulose, an amount of glycerin equal to substantially 4% or less of the weight of the nitrocellulose and an 50 amount of water equal to substantially 4% or less of the weight of the nitrocellulose.

9. A flowable film-forming composition of matter comprising nitrocellulose, a volatile common solvent, an amount of a sugar

equal to approximately 4% or less of the weight of the nitrocellulose, an amount of an inert hygroscopic organic compound of low volatility equal to substantially 4% or less of the weight of the nitrocellulose and an amount of water equal to substantially 4% or less of the weight of the nitrocellulose.

10. A flowable film-forming composition of matter comprising nitrocellulose, a volatile common solvent, an amount of a sugar 65 equal to approximately 4% or less of the weight of the nitrocellulose, an amount of glycerin equal to substantially 4% or less of the weight of the nitrocellulose and an amount of water equal to substantially 4% or less of the weight of the nitrocellulose.

11. A flowable film-forming composition of matter comprising nitrocellulose, a volatile common solvent, an amount of glucose 75 equal to substantially 4% or less of the weight of the nitrocellulose, an amount of an inert hygroscopic organic compound of low volatility equal to substantially 4% or less of the weight of the nitrocellulose and an amount of water equal to substantially 4% or less of the weight of the nitrocellulose.

12. A flowable film-forming composition of matter comprising nitrocellulose, a volatile common solvent, an amount of glucose 85 equal to substantially 4% or less of the weight of the nitrocellulose, an amount of glycerin equal to substantially 4% or less of the weight of nitrocellulose and an amount of water equal to substantially 4% or less 90 of the weight of the nitrocellulose.

13. A composition of matter comprising 100 parts of nitrocellulose, 200 to 400 parts of acetone, 200 to 400 parts of methyl alcohol, 20 to 200 parts of a monohydroxy aliphatic alcohol having from 4 to 5 carbon atoms, 1 to 30 parts of camphor, and an amount of each of the following ingredients equal to substantially 4 parts or less,—glucose, glycerin and water.

14. The process of modifying a flowable film-forming nitrocellulose dope, which comprises pre-mixing glucose, glycerin and water and then incorporating the mixture with said dope.

Signed at Rochester, New York, this 6th day of April, 1921.

PAUL C. SEEL.

100

105